

C. H. URQUHART.

PROCESS OF PRECIPITATING AND RECOVERING METALS.  
APPLICATION FILED SEPT. 9, 1913.

1,090,661.

Patented Mar. 17, 1914.



Witnesses  
A. Christensen  
C. L. Pamelle

Inventor

Charles H. Urquhart

By  
George W. Bruce  
Attorney

# UNITED STATES PATENT OFFICE.

CHARLES H. URQUHART, OF NEWARK, NEW JERSEY.

## PROCESS OF PRECIPITATING AND RECOVERING METALS.

1,090,661.

Specification of Letters Patent. Patented Mar. 17, 1914.

Continuation of application Serial No. 775,165, filed March 18, 1913. This application filed September 9, 1913. Serial No. 788,893.

*To all whom it may concern:*

Be it known that I, CHARLES H. URQUHART, a citizen of the United States, and a resident of the city of Newark, in the county 5 of Essex, State of New Jersey, have invented certain new and useful Improvements in the Process of Precipitating and Recovering Metals, of which the following is a specification.

10 This invention relates to metallurgical processes and more particularly to a process of recovering precious metals, especially gold and silver, from cyanid solutions.

The principal object of this invention is 15 the recovery of precious metals in solution, by passing the solution through granulated zinc, and excluding the air from the granulated zinc during the passage of the solution.

20 Another object of this invention is the recovery of precious metals by passing the pregnant solution through granulated zinc, excluding air from the zinc, and agitating the mass, thereby causing the particles of 25 the precious metals to be freed from the zinc and at the same time breaking up the granulated zinc to produce clean unoxidized surfaces for further carrying on the process of precipitation.

30 Still other and further objects of this invention will in part be obvious, and will in part be pointed out in the specification hereinafter following by reference to the accompanying drawings.

35 This application is a continuation of my prior application bearing Serial No. 775,165, and filed March 18, 1913.

The figure of the drawing illustrates a 40 preferred form of apparatus in which my process may be carried out. There may be other forms of devices, however, in which my process may be conducted.

Metallic zinc has long been known as 45 being a good precipitant for precious metals from cyanid solutions, but its use heretofore has been attended with many difficulties. Zinc threads or shavings have been used, but the cost thereof is high, and even when packed tightly in boxes (the boxes are 50 arranged in a stepped tandem series to suc-

cessively treat the metal bearing solution) the shavings soon become polarized and coated and require frequent washing in order to enable the process to be continued with any degree of success. In practice the 55 zinc shavings must be handled daily (in some mills weekly) thereby entailing considerable manual labor. In the operation of the zinc shavings boxes there are formed what are known in the art as "zinc shorts." 60 These "zinc shorts" constitute small particles of zinc broken off from the shavings, and they settle to the bottom of the box thereby becoming covered with the precipitates and consequently are inactive. Furthermore, in the subsequent smelting of the precipitates, these "zinc shorts" are very detrimental in that they incur considerable expense by requiring a large amount of flux to be used. This difficulty is well known in 70 the art, and it is customary, in order to obviate it, to give the precipitate containing "zinc shorts" a preliminary treatment with sulfuric acid to dissolve out the zinc. This treatment is, of course, expensive; further- 75 more, the repeated handlings necessary mean a certain loss of the precious metals. It also happens, in the use of the zinc shavings box process, that a large percentage of the precipitate clings to the coarse zinc par- 80 ticles in the box and consequently is not recovered during the ordinary working of the process. Zinc dust has also been used (known as "zinc fume"), but even this has 85 many disadvantages. The zinc dust is costly. It must be stored and shipped in hermetically sealed containers, and as soon as a container is broken or opened the contents thereof must be used, otherwise the dust will oxidize, and oxidized zinc in a 90 cyanid solution is very undesirable and detrimental. The extreme liability of "zinc fume" to oxidize renders it inflammable and explosive and therefore dangerous to handle and expensive to ship. This feature alone 95 is of importance because most precious metal mines are more or less isolated and the question of shipping supplies is of great importance commercially. Zinc spheres in the form of shot have also been used as pre- 100

cipitants, but the smooth surfaces of the spheres do not constitute good surfaces for causing the forming and effusion of hydrogen. The smooth surfaces are not the best 5 sort of surfaces to carry on electro-chemical reactions.

In the commercial treatment of large quantities of metal bearing solution, to recover the precious metals therefrom there 10 are two things that are especially desirable; first, a satisfactory precipitant, capable of being economically obtained, easy to transport, and safe to handle; second, a substantially continuous process for using said precipitant, said process requiring a minimum 15 amount of manual labor, and skilled attendants, to carry out the process, and keep the precipitant in working condition. I have discovered by experiment and study that 20 granulated zinc, prepared as described below, satisfies the first mentioned requirement, and that treatment of the pregnant solution by passing the same through a mass of the granulated zinc in a closed chamber 25 entirely filled with solution, thereby excluding the air, and agitating the granulated zinc so as to grind or remove the precipitated metal and form minute zinc particles, satisfies the second requirement, for the reason 30 that when the process is so carried out it is unnecessary to re-handle the granulated zinc, and the whole process is continued, or carried out, entirely by machinery instead 35 of manual labor, and it does not require skilled attendants. And my process is free from the difficulties I have above referred 40 to in connection with the art prior to my invention.

The granulated zinc, to which I have referred as a precipitant, is prepared by melting common pig zinc, known in the art as "spelter," heating the melted zinc to a high temperature, but not sufficient to volatilize the same, then pouring the melted zinc from 45 a height of 2 or 3 feet into a bath of cold water. The resulting product comprises comparatively small, irregular, unoxidized masses of brittle zinc. This product is cheap to produce and may be handled without danger, since it is not inflammable nor explosive. Its irregular form affords a mass of zinc 50 having ideal surfaces for precipitation purposes, and for enabling the hydrogen to freely form and escape. The granulated zinc produced in the manner prescribed, is not malleable, but is so brittle that when introduced into a revolving drum it breaks up into minute particles by attrition, without the use of abrasives, or without the 55 necessity of mixing other metals with the zinc to form a special alloy to secure the brittle product. Where metals are used to alloy the zinc to secure brittleness, these 60 metals may not act as precipitants, but they

do go into solution, and to this extent tend 65 to use up, or foul, the cyanid solution, and the alloy is, of course, more expensive to produce than is the simple metal.

The term "granulated zinc" is sometimes loosely used to designate small round, or 70 substantially round, particles of zinc commonly called "shot zinc". The product which I have herein designated as "granulated zinc" should not be confused with shot zinc. Shot zinc is formed by permitting molten zinc at a comparatively low 75 temperature, to fall into water from a height sufficient to permit the particles to form into globules or spheres before they reach the water. To permit the globules or 80 spheres to retain their form it is necessary that they be sufficiently cooled by falling through the air to prevent their being broken or shattered when they strike the water. It will therefore be seen that shot 85 zinc is not subjected to a sudden and extreme chill when the metal reaches the water. My granulated zinc on the contrary, as prepared as above specified, results from a very hot and fluid metal striking a chilling bath after a short fall. The metal being very limpid tends to "spread out" or 90 "splash" when it strikes the cold water, the result being that the thin layer of metal is thus formed into highly crystalline and brittle flakes of irregular conformation. The irregular formation of this material renders it especially good for electro-chemical action and it thereby forms a splendid precipitating medium. The highly crystalline 95 character of the particles renders the material very brittle so that when tumbled *en masse* in a revoluble drum the particles break and thus continuously form new surfaces for deposition of the precious metals. 100 This breaking up of the particles is far more desirable and operates far more effectively than where masses of zinc are subjected to the action of an abrasive to secure new surfaces. The action of an abrasive is never 105 entirely perfect, whereas a break in the material leaves an absolutely clean crystalline surface for further activity.

In the treatment of the pregnant solution with zinc, it is necessary to practical success 115 that no air be present, and therefore, I have found it convenient to carry out the process in the following apparatus, which I will describe by referring to the drawings:—

The granulated zinc is carried in the revolving drum 1 and is introduced therein through the hand hole 2. The revolving drum is provided at each end with headers 4, which carry screens 5 and 6, indicated diagrammatically in the drawings. These 120 screens are for the obvious purpose of retaining the granulated zinc within the drum 1. Tubular shafts 7 and 8 are respectively

carried by the headers 4, and when in position in the bearings 9 and 10, constitute the supports for the drum 1, and also constitute ducts or conduits through which the 5 pregnant solution is introduced into the drum. The tubular shaft 7 carries a large gear 11, which, coöperating with a suitable driving gear, not shown, comprises a means for rotating the drum to agitate the 10 contents thereof.

The shaft 7 terminates within a vertical inlet well 12, and a stuffing box, or gland, 14, is provided to insure a running fluid tight joint where the shaft 7 enters the said well 15 12. This well 12 is provided with a suitable cleanout pipe 15. The shaft 8 terminates within an outlet well 16, which likewise is provided with a stuffing box 17, to also insure a fluid tight running joint. The outlet 20 well 17 is provided, near the upper end thereof with an outlet pipe 18, and is provided at the lower end with a suitable cleanout pipe 23. The lowest part of the opening in the outlet pipe 18 is in a horizontal line 25 slightly above the highest part of the interior of the drum 1, which highest part is at the hand hole 2 when the drum is in the position indicated in the drawings.

In order to carry out my process the granulated zinc is prepared as I have specified, 30 the drum is revolved until the hand hole is at the highest position, as indicated by the drawings, the hand hole cover removed, and the drum partly filled with the granulated zinc. The pregnant solution is then run 35 into the inlet well 12, and, of course, from the well into the drum 1 until the drum is entirely filled. The filling of the drum will take place before any solution will flow out 40 of the outlet pipe 18 for the reason that, as has been explained, this outlet pipe is slightly higher than the highest point in the drum. The hand hole cover is then replaced and the apparatus is ready to carry out the 45 process.

As the drum 1 is slowly revolved by the gear 11, and coöperating driving mechanism, the brittle granulated zinc will be broken up by abrasion or attrition. The breaking up 50 of the brittle zinc particles takes place under the solution within the revolving drum 1, from which the air is entirely excluded, and therefore produces small particles of zinc having clean, fresh, irregular surfaces which 55 are entirely free from oxid since they are produced free from oxidizing conditions. The process may be carried on substantially continuously, it only being necessary to occasionally add granulated zinc to the drum 60 to take the place of such zinc particles as are consumed. The abrading action of the zinc particles frees the precipitated precious metal, gold or silver, which for the greater part is carried off by the solution in suspen-

sion and may be removed by any suitable device. For example, the outlet pipe 18 may discharge into a settling tank 19, provided with baffles 20, and having a sloping bottom 21, where the most of the precipitated metal will settle and from which it may be removed from time to time by the cleanout valve 22, or in any other convenient manner. The solution may pass into a further chamber 24 partly filled with a coarse precipitating and filtering material, and may eventually pass into a still further filtering chamber 25 which is preferably charged with a combustible filtering material. The final clear liquor is conveniently drawn off through a proper pipe or duct 26 and may 80 then be used for another cycle of operations.

Since the invention as set forth herein relates entirely to a process, I desire it to be understood that the apparatus illustrated and described is merely for illustrative purposes, and that my process may be carried out in many widely different sorts of devices which specifically form no part of the present invention.

Whenever the term "zinc" is used herein 90 it is intended also to include commercial zinc, known in the art as "spelter."

Having thus described my invention what I claim is,—

1. The process of precipitating and recovering metals from solution, which consists in passing the pregnant solution into and through a mass of specified granulated zinc in a closed chamber, the pregnant solution entirely filling the said chamber, thereby excluding air from the granulated zinc; agitating the solution and granulated zinc to free the precipitated metals from the zinc by abrasion; then separating the free metal particles from the solution. 95

2. The process of precipitating and recovering metals from solution, which consists in submerging a mass of specified granulated zinc by the pregnant solution; comminuting the granulated zinc while so submerged, 100 thereby also freeing the precipitated metal; and then recovering the free metal from solution. 105

3. The process of precipitating and recovering metals from solution, which consists in submerging a mass of specified granulated zinc by a substantially continuous flow of pregnant solution; agitating the mass of granulated zinc during the flow of the pregnant solution to free the precipitated metal, 115 then recovering the free metal from the solution. 120

4. The process of precipitating and recovering metals from solution, which consists in passing the solution through granulated zinc 125 repaired as specified; excluding air from said granulated zinc during the passing of said solution; agitating said granulated zinc

to produce a grinding action between the particles; then separating the free metal particles from the solution.

5. The process of precipitating and recovering metals from solution, which consists in passing the metal bearing solution into a mass of granulated zinc repaired as specified; excluding air from said granulated

zinc when the solution is present; agitating the granulated zinc to remove the precipitated metals by abrasion; then separating the free metal particles from the solution. <sup>10</sup>

CHARLES H. URQUHART.

Witnesses:

GEORGE W. RAMSEY,  
EDITH C. RAMSEY.